

## UNITED STATES PATENT OFFICE

CONWAY, BARON VON GIRSEWALD, AND HANS WEIDMANN, OF FRANKFORT-ON-THE-MAIN, GERMANY, ASSIGNEES TO AMERICAN LURGI CORPORATION, OF NEW YORK, N. Y., A CORPORATION OF NEW YORK

PROCESS FOR THE CONVERSION OF FERRO-PHOSPHORUS INTO FERRIC PHOSPHATE (FePO<sub>4</sub>) BY ROASTING IN AIR OR OTHER GASES CONTAINING OXYGEN

No Drawing. Application filed May 5, 1930, Serial No. 450,058, and in Germany May 29, 1929.

This invention relates to a process for the conversion of ferro-phosphorus into ferric phosphate (FePO<sub>4</sub>) by roasting in air or other gases containing oxygen. Considerable difficulties are encountered in carrying out this process, since the oxidation is extremely slow. If, for example, finely ground ferro-phosphorus having a phosphorus content of 24% is roasted in accordance with the usual methods in a muffle furnace at temperatures of for example, 700 to 800° C., it is only possible, even in the presence of large amounts of moist air, to convert about 16% of the initial material into ferric phosphate during a roasting period of 10 hours.

It has been found in accordance with the present invention that the oxidation process can be catalytically accelerated. Alkali metal compounds such as common salt or soda may advantageously be employed as catalysts. The catalytic action of such substances becomes already noticeable if the same are present in relatively small amounts of for example, 1% and less. Nevertheless, larger amounts of catalytically acting additional substances may be employed according to requirements. Salts of alkaline earth metals such as for example, calcium chloride may also be employed as catalysts. Moreover, it is possible to employ several catalysts in conjunction such as for example, an alkali metal salt and an alkaline earth metal salt.

*Example*

5 kilograms of ferro-phosphorus containing 24% P are mixed in a finely ground state with 50 grams of sodium chloride, and the mixture is roasted in a muffle furnace at 700 to 800° C., in the presence of air. After a roasting period of only 6 hours, 85% of the ferro-phosphorus had been converted into ferric phosphate. At the end of the roasting process, traces only of chlorine can be detected in the roasted material.

In general, it has been found that the moisture present in the air is sufficient, and consequently it is not necessary as a rule to increase the degree of humidity of the air.

We claim:

1. A process for the production of ferric

phosphate which comprises treating ferro-phosphorus at elevated temperature with oxygen-containing gases in the presence of a substance of the group consisting of alkali and alkaline earth metal compounds.

55

2. A process for the production of ferric phosphate which comprises treating ferro-phosphorus at elevated temperatures with air in the presence of a relatively small amount of a compound of the group consisting of the water-soluble alkali and alkaline earth metal compounds.

60

3. A process for the production of ferric phosphate which comprises treating ferro-phosphorus at elevated temperatures with oxygen-containing gases in the presence of an alkali metal compound.

65

4. A process for the production of ferric phosphate which comprises treating ferro-phosphorus at elevated temperatures with oxygen-containing gases in the presence of a sodium compound.

70

5. A process for the production of ferric phosphate which comprises treating ferro-phosphorus at elevated temperatures with oxygen-containing gases in the presence of sodium carbonate.

75

6. A process for the production of ferric phosphate which comprises treating ferro-phosphorus at elevated temperatures with air in the presence of a relatively small amount of a water-soluble alkali metal compound.

80

7. A process for the production of ferric phosphate which comprises treating ferro-phosphorus at elevated temperatures with air in the presence of a relatively small amount of sodium chloride.

85

In testimony whereof, we affix our signatures.

CONWAY BARON von GIRSEWALD.  
HANS WEIDMANN.

90

95

100